

# UNITED STATES PATENT OFFICE.

KOTARO HONDA, OF YONEGA-FUKURO, SENDAI, JAPAN, ASSIGNOR TO SUMITOMO CHUKOSH, LTD., OF OSAKA, JAPAN, A CORPORATION OF JAPAN.

## MAGNET-STEEL.

1,338,132.

Specification of Letters Patent. Patented Apr. 27, 1920.

No Drawing.

Application filed October 22, 1917. Serial No. 197,837.

To all whom it may concern:

Be it known that I, KOTARO HONDA, D. Sc., citizen of Japan, residing at No. 21 Kanoko Shimidzu, Yonega-fukuro, Sendai, Japan, have invented certain new and useful Improvements in Magnet-Steel; and I do hereby declare the following to be a full, clear, and exact description of the invention, such as will enable others skilled in the art to 10 which it appertains to make and use the same.

This invention relates to novel magnet steels and to magnets made therefrom. More particularly, the invention relates to the manufacture of permanent magnets from alloys comprising carbon steel, cobalt, and one or more metals of the chromium family. Magnets made in accordance with the invention materially excel magnets heretofore 20 known especially in point of strong residual magnetism and large coercive force.

In the particular embodiment of the invention here chosen for purposes of illustrating and explaining the broad principles involved, tungsten is the particular metal of the chromium group constituting an essential ingredient of the alloy, the use of chromium in addition to tungsten being very desirable but not essential. In my copending 30 application, Serial No. 197,838, filed October 22, 1917, is disclosed and claimed another specific embodiment of the invention in which chromium is the only metal of the chromium group specified as an essential ingredient of the magnet steel in question; while in another copending application Serial No. 197,839, filed October 22, 1917, is disclosed and claimed another specific embodiment of the invention in which molybdenum, and optionally chromium, are specified as ingredients of the alloy steel.

In a typical instance, a magnet embodying the principles of the invention may be made of an alloy steel having the following 45 range of composition:

Cobalt, 5-60%; tungsten, 1-10%; chromium, 0.5-10%; carbon steel, (with 0.5-2% carbon,) the remainder. Most desirably the cobalt content is from 20 to 60%, and 50 has been found particularly suitable. The chromium, although a desirable constituent, may be omitted without seriously diminishing the magnetic property of the alloy. Other elements commonly present in steel

may also be present in the alloy, and vanadium or the like may also be added.

In manufacturing this alloy steel, a mixture of the above-mentioned metallic ingredients may be melted at a temperature of, say 1700° to 1800° C., and poured to 60 form an ingot. When sufficiently cooled the ingot is forged and worked into the form of a magnet, and is then hardened as by quenching at a temperature of say around 1100° C., for example, this temperature being considerably higher than the quenching temperature for ordinary magnet steel which is about 800° C. After quenching, the shaped body of paramagnetic metallic material is strongly magnetized with the aid of 70 a powerful magnet or coil.

The magnet produced in the manner described is far superior to magnets heretofore known in the art, particularly as regards—

(1) Coercive force which in magnets of 75 the best type heretofore known does not exceed 75 C. G. S. units, whereas in the present magnet, the specific coercive force reaches 200 C. G. S. units. For this reason, loss of magnetism or so-called magnetic decay, due 80 to shock or lapse of time is exceedingly small in the case of the present magnet.

(2) Intensity of magnetization per unit volume, which in the known magnets of the best type rarely exceeds 450 C. G. S. units 85 after artificial aging; whereas owing to its large coercive force the intensity of magnetization of the present magnet commonly exceeds 700 C. G. S. units after artificial aging.

The foregoing remarkable distinguishing characteristics of my new magnet obviously render the same capable of wide use to an increased extent in arts in which the magnet plays an important part.

What I claim is:

1. A method of preparing permanent magnets which comprises quenching a body of paramagnetic alloy steel containing cobalt at a temperature substantially above 100 800° C., and thereafter magnetizing the same.

2. The method of preparing permanent magnets which comprises quenching a body of an alloy steel containing from about 5 to 105 60 per cent. cobalt, from about 1 to 10 per cent. tungsten, and from about 0.5 to 10 per cent. chromium, at a temperature substan-

tially above 800° C., and thereafter magnetizing the same.

3. The method of preparing permanent magnets which comprises quenching a body of an alloy steel containing cobalt and a metal of the chromium group at a temperature approximating 1100° C., and thereafter magnetizing the same.

4. The method of preparing permanent magnets which comprises quenching at a temperature substantially above 800° C. a body of an alloy steel containing cobalt and a metal of the chromium group, and thereafter magnetizing said body.

15 5. The method of preparing permanent magnets which comprises quenching at a temperature substantially above 800° C. a body of an alloy steel containing cobalt and tungsten and thereafter magnetizing said body.

20 6. The method of preparing permanent magnets which comprises quenching at a temperature substantially above 800° C. a body of an alloy steel containing cobalt, tungsten and chromium, and thereafter magnetizing said body.

25 7. In a method of preparing permanent magnets, the step which comprises quenching a body of paramagnetic alloy steel containing cobalt at a temperature substantially above 800° C.

30 8. In a method of preparing permanent magnets, the step which comprises quenching a body of an alloy steel containing cobalt and a metal of the chromium group, at a 35 temperature approximating 1100° C.

9. As a new article of manufacture, a magnetized body of an alloy steel containing cobalt and a metal of the chromium group.

40 10. As a new article of manufacture, a magnetized body of an alloy steel containing cobalt and tungsten.

11. As a new article of manufacture, a magnetized body of an alloy steel containing cobalt, tungsten and chromium.

45 12. As a new article of manufacture, a permanent magnet made of an alloy containing from about 5 to 60 per cent. cobalt, from about 1 to 10 per cent. tungsten, and 50 carbon steel of from about 0.5 to 2 per cent. carbon.

55 13. As a new article of manufacture, a permanent magnet made of an alloy containing from about 5 to 60 per cent. cobalt, from about 1 to 10 per cent. tungsten, from about 0.5 to 10 per cent. chromium, and carbon steel of from about 0.5 to 2 per cent. carbon.

60 14. As a new article of manufacture, a permanent magnet comprising a magnetized body of an alloy steel containing from 5 to 60 per cent. cobalt substantially uniformly distributed therethrough.

65 15. As a new article of manufacture, a permanent magnet comprising a magnetized body of an alloy steel containing a substantial percentage of cobalt substantially uniformly distributed therethrough.

70 In testimony whereof I hereunto affix my signature.

KOTARO HONDA.